

## UNITED STATES PATENT OFFICE

2,198,775

## FERROUS ALLOY

Walter E. Jominy, Detroit, Mich., assignor to  
General Motors Corporation, Detroit, Mich., a  
corporation of Delaware

No Drawing. Application November 5, 1938,  
Serial No. 239,022

6 Claims. (Cl. 75—126)

This application relates to ferrous alloys and more particularly to cast iron compositions which have very good properties of wear resistance. The alloys forming the subject matter of the present invention possess the resistance to scoring characteristic of cast iron and have extra good properties as regards resistance to wear under severe conditions. The alloys in accordance with my invention are especially adapted for such parts as cylinder liners, piston rings, pistons, valves, valve guides, tappets, bearings and other parts ordinarily subjected to wear.

The invention comprises alloys composed of carbon, silicon, titanium, copper, manganese, chromium, and iron as essential constituents. Ordinary impurities as sulphur, phosphorus, etc., are present in small amounts. For example, the sulphur is usually present from a trace up to .12%. In some cases slightly greater amounts, say up to .20% may be present without unduly affecting the beneficial effects of the essential constituents. The phosphorus is ordinarily kept low, that is, under about .20%. However, higher amounts up to about 1% may be present.

The several essential constituents are in approximately the following proportions: 2.25-4.00% carbon, 1.50-3.50% silicon, .05-60% titanium, .50-1.50% copper, .30-1.00% manganese, .40-2.00% chromium, balance iron.

A preferred narrower range of the essential ingredients is the following: 2.75-3.75% carbon, 2.00-3.20% silicon, .10-.45% titanium, .55-1.10% copper, .40-80% manganese, .50-1.25% chromium, balance iron.

In addition to the ability to resist scoring and wear, the alloys of my invention are ordinarily comparatively easy to machine. It will be understood by those skilled in the art that the carbon and silicon content may be modified within the ranges given to suit the casting size and/or cooling rate in order to obtain extremely good machinability. It is common knowledge in the field of metallurgy that small castings by reason of their faster cooling will have more combined carbon and less graphitic carbon than will castings of large size when both are made of the same chemical composition. Higher combined carbon and less graphitic carbon will make machining more difficult so that the composition must be modified to compensate for this condition. This may be done by adding more silicon, more carbon, or more of both silicon and carbon.

Within the range of composition given it is possible in certain section sizes to obtain white

cast irons which would, of course, be rather difficult to machine.

There are many instances when other specific properties in addition to the ability to resist wear are required in a cast iron. Such a property as high strength in larger size castings, as well as good hardness near the center of large castings, is frequently essential. Also, in many cases it is highly desirable that the iron have extra good fluidity at ordinary casting temperatures and/or be easily melted in the cupola. In many cases it is highly desirable that the casting be leak resistant.

The following compositions having the essential constituents in approximately the proportions stated have been found especially good as regards resistance to wear. In bars  $\frac{3}{8}''$  x  $\frac{1}{8}''$  x 12" cast in green sand molds these compositions are readily machinable. The several examples given each have good resistance to wear and allow some variation in other desirable physical properties.

*Example No. 1*

2.86% carbon, 2.18% silicon, .16% titanium, .94% copper, .62% manganese, .51% chromium, balance iron. 25

*Example No. 2*

3.17% carbon, 2.29% silicon, .14% titanium, .58% copper, .74% manganese, .58% chromium, balance iron. 30

*Example No. 3*

3.26% carbon, 2.61% silicon, .28% titanium, .99% copper, .65% manganese, 1.13% chromium, balance iron. 35

*Example No. 4*

2.90% carbon, 2.38% silicon, .26% titanium, 1.05% copper, .49% manganese, 1.19% chromium, balance iron. 40

*Example No. 5*

3.26% carbon, 2.61% silicon, .28% titanium, .99% copper, .65% manganese, 1.13% chromium, .76% phosphorus, balance iron. 45

The several alloying constituents may be incorporated in any convenient manner. As regards titanium, one convenient method of adding the same is in the form of a silicon titanium alloy. In order to reduce the tendency of the titanium to become oxidized, it is preferably added at a late stage in the melting process. If desired to add silicon late to get higher strength it is permissible. Any suitable melting furnace may be used. 50

I claim:

1. An alloy comprising the following elements as essential constituents in approximately the amounts stated: 2.25-4.00% carbon, 1.50-3.50% silicon, .05-.60% titanium, .50-1.50% copper, .30-1.00% manganese, .40-2.00% chromium, balance substantially all iron.
2. An alloy composed of the following elements as essential constituents in approximately the amounts given: 2.75%-3.75% carbon, 2.00-3.20% silicon, .10-.45% titanium, .55-1.10% copper, .40-.80% manganese, .50-1.25% chromium, balance iron.
3. An alloy composed of the following elements as essential constituents in approximately the proportions given: 2.86% carbon, 2.18% silicon, .16% titanium, .94% copper, .62% manganese, .51% chromium, balance iron.
4. An alloy composed of the following elements as essential constituents in approximately the proportions given: 3.17% carbon, 2.29% silicon, .14% titanium, .58% copper, .74% manganese, .58% chromium, balance iron.
5. An alloy composed of the following elements as essential constituents in approximately the proportions given: 2.90% carbon, 2.38% silicon, .26% titanium, 1.05% copper, .49% manganese, 1.19% chromium, balance iron.
6. A cast iron alloy containing 2.25-4.00% carbon, 1.50-3.50% silicon, .05-.60% titanium, .50-1.50% copper, .30-1.00% manganese and .40-15.200% chromium.

WALTER E. JOMINY.